

# UNITED STATES PATENT OFFICE.

FRANÇOIS LAMY, FILS, OF DEVILLE-LES-ROUEN, FRANCE.

## IMPROVEMENT IN DYEING FABRICS WITH NAPHTYLAMINE COLORS.

Specification forming part of Letters Patent No. 134,076, dated December 17, 1872.

*To all whom it may concern:*

Be it known that I, FRANÇOIS LAMY, *Fils*, of Deville-les-Rouen, in the Republic of France, do hereby declare the nature of my said invention for Improvements in the Production of a puce-garnet color or colors from Naphthylamine and its derivatives, of which the following is a description:

My invention has for its object the production, at a less cost than hitherto, of colors of puce-garnet, violet, and reddish-violet tints in such a manner as to preserve the solidity of the substances of pure madder.

Hitherto certain colors, such as red, violet, puce, reddish violet, orange, and similar colors were produced almost exclusively either by dyeing, with previous oxidation of the mordants, by means of madder, flower of madder, and analogous products, or by application and vaporizing without oxidation of mordants by means of extracts of madder. Moreover, and in proportion to the value of the result determined by the operator, to the said dyeing materials were often added different products, such as wood in powder, certain astringents, or extracts of wood. By thus reducing the value of the result the degree of solidity of the coloring matter fixed on the fabric was diminished.

It has therefore been my object to produce, at an equal if not at a lower cost, some of the shades of color mentioned above, while still maintaining the solidity, as it were, absolutely, of the substances of pure madder, and I have discovered, first, a solid puce depending on the normal limits of the value of the result. And it is this mode of proceeding or operation that constitutes the object of the present invention. For this purpose I utilize the properties possessed by certain products of forming fixed bases, and particularly naphthylamine, a product obtained from naphthaline, transformed at first into nitro-naphthaline, then distilled on iron filings.

After dissolving the naphthylamine in a mixture of azotic or hydrochloric acid and acetic acid, I treat it with chloric and chromic acid in the following manner: I take a salt of naphthylamine, nitrate, acetate, or hydrochlorate. I suitably thicken it; then I add in the color oxidizing salts, such as chlorate of potash,

salts of copper, salts of iron, as well as hydrofluosilicic acid. After printing, I spread out the pieces of fabric in a room for some time, exposed to the air; then I fix the color by passing them into a bath of bichromate of potash in which I have added a certain proportion of nitric or sulphuric acid or hydrochloric acid. Finally, in order to develop the puce shade of color, I add a passing into chlorine (by preference an alkaline chloride) or into ammonia. I thus obtain a puce possessed of a great solidity, and which presents, as will be seen, nearly the same characteristics as aniline black.

For dyeing on threads or fibers of cotton or silk, separate or in skeins, I make use of the same elements; only, instead of operating on them in drying, I operate by a wet process—that is to say, by dipping.

The puce-garnet obtained by this process may be considered as a mother color, which, by slight modifications in its constituent elements or by subsequent operations, admits of the production of derivative colors, of which the principal base is always naphthylamine.

Thus, with reference to dyeing threads or fibers of cotton or silk, if, instead of finishing by passing through ammonia and chlorine in order to develop the tint, the threads or fibers are passed into a bath composed of azotate of iron and *aqua regalis*, (a mixture of hydrochloric acid and nitric or azotic acid,) a beautiful violet is obtained. By substituting, in the last-mentioned bath, for the azotate of iron, chloride of iron and a salt of copper a reddish violet is obtained.

These two tints or shades of color, perfectly distinct and derived from the same base, are possessed of great solidity as to acids, alkalies, and solar light.

My discovery consists, then, in fixing, by a regular and practical method, on silk and cotton, naphthylamine, a product known for a long time, but which, up to the present time, could only be utilized in making the said rose-tint of naphthylamine.

This latter product is employed in dyeing on wool and silk, or for making certain colors, such as a violet and a gray, for printing on cotton; but these last colors are wanting in solidity against the light, and have been but little, if at all, applied up to this time.

These colors equal in intensity those obtained with madder and its derivatives on a mordant of alumina, of iron, or of chromium, and are equal if not superior to them in solidity.

Having thus described the nature of the said invention, and the mode of carrying it into effect, I hereby declare that what I claim as of my invention is—

The production on cotton and silk, by means of the three processes above described, of the three tints or shades of color, being a puce-garnet, a violet, and a reddish violet.

F. LAMY, *Fils.*

Witnesses:

B. DAVOUST,  
PREVOST.